# EUROPEAN PATENT SPECIFICATION

(11) **EP 3 812 056 B1**
(45) Date of publication and mention of the grant of the patent: **04.02.2026**
(21) Application number: 19838335.8
(22) Date of filing: 09.07.2019
(51) Int. Cl.: B21B 17/04, B21C 37/06

(54) **PREPARATION METHOD FOR A MEDIUM/SMALL-DIAMETER THICK-WALLED METAL TUBE**
VERFAHREN ZUR HERSTELLUNG EINES DICKWANDIGEN METALLROHRES MIT MITTLEREM/KLEINEM DURCHMESSER
PROCÉDÉ DE FABRICATION D'UN TUBE MÉTALLIQUE À PAROI ÉPAISSE ET DE PETIT OU MOYEN DIAMÈTRE

(30) Priority: 17.07.2018 CN 201810783775
(43) Date of publication of application: 28.04.2021
(73) Proprietor: Han, Jingtao, Beijing 100083 (CN)
(72) Inventor: HAO, Qingle, Beijing 100083 (CN); HAN, Jingtao, Beijing 100083 (CN)
(74) Representative: Grünecker Patent- und Rechtsanwälte PartG mbB
(86) International application number: PCT/CN2019/095282
(87) International publication number: WO 2020/015556

(56) References cited:
- CN-A- 101 249 603
- CN-A- 101 633 115
- CN-A- 104 475 479
- CN-A- 104 475 479
- CN-A- 105 710 273
- CN-U- 208 495 380
- CN-U- 208 695 986
- GB-A- 1 092 718
- US-A- 2 247 863
- US-A- 3 404 449

## Description

### Technical Field

The invention involves the technical field of metal tube material processing. More in detail, the invention relates to a preparation method for a medium-small-aperture thick-wall metal tube (see e.g. US 2 247 863 A).

### Background Art

At present, the method for forming the medium-small-aperture thick-wall (D/S is in the range of 2-20) metal tube mainly comprises extrusion, rolling, and the like. The extrusion forming production efficiency is low so that the product cost is high, the market competitiveness is not achieved, and the method is generally used for producing very few metal tubes which cannot be or are difficult to produce by other processes. Hot rolling forming mainly includes periodic tube rolling, three-roller skew rolling forming and tension-reducing forming.

The rotary forge mill feeds the tubing into a rolling groove composed of a mandrel and a periodic reciprocating moving roll-pass at a certain frequency. The inner wall of the tube is supported by the mandrel, and the tube blank is rolled by a gradually shrinking variable-cross-section roll-pass so that the functions of reducing the diameter and reducing the wall are realized. The common rotary forge mill is mainly the two-roller pilger mill. However, due to the reciprocating movement of the rack and the rollers during the rolling process, many moving parts are needed and the inertia is large, the stability of the rolling process is poor, the structure of the rolling mill is complicated, and the maintenance and adjustment are difficult; the tubing rolled by the two-roller rolling mill has low dimensional accuracy and poor surface quality.

The three rollers of the three-roller skew rolling mill are uniformly distributed around the rolling center line at 120 degrees, and the axes of the rollers and the rolling center line are inclined and crossed to form a certain angle (i.e. a rolling angle and a feeding angle), so that the tube blank spirally advances under the action of the rollers, and the outer surface of the rolled tubing can form a "spiral line", influencing the surface quality, and the rolling jamming being caused by a "triangular" defect which easily appears at the tail part.

A three-roller tension reducing mill generally comprises more than 10 racks to form a series of roll-passes. Tension is provided through the speed difference of the rotating speeds of rollers of adjacent racks, so that hollow reducing of the tube blank is completed. But due to a large number of racks, the equipment investment is large, the production line is long, the occupied area is large, and the equipment adjustment and control are complicated.

### Summary of the Invention

In order to solve the problems in the prior art, the invention provides a preparation method for a medium/small-aperture thick-wall metal tube, according to claim 1. The invention has the characteristics of forging and rolling, can realize single pass and large deformation amount processing of the metal tube blank, and has the advantages of short process flow, high product dimensional accuracy (±0.2mm), good quality of the inner wall and outer wall surface and low cost.

A medium-small-aperture thick-wall metal tube thereby obtained, has a cross-sectional diameter from 30mm to 160mm, a dimensional accuracy of ±0.2mm, and a ratio of an outer diameter of the metal tube to a wall thickness of the metal tube greater than 2 to less than or equal to 20.

Preferred embodiments are defined in the dependent claims.

When cold forming is carried out, the tube blank is fed and then directly fed into a composite forging and rolling forming device; when hot forming is carried out, the blank is heated to a target temperature , preferably of 800° to 1200°C, through an induction heating device and then fed into the composite forging and rolling forming device.

Preferably, the blank selected in the invention comprises a high-frequency longitudinal welded tube and a seamless tube, the material requirement comprises a steel tube and nonferrous metal tubes such as aluminum, copper, magnesium and titanium and the like, the outer diameter of the tube blank is 40-180mm, and the cut length is 0.5-10m.

As already mentioned, the process can be used for cold forming and hot forming. When hot forming, an induction heating device is foreseen in step (3), e.g. a medium-frequency induction heating coil, and the forming temperature range is 800-1200° C**.**

The beneficial effects of the above-mentioned technical scheme provided by the invention are as follows:
(1) the single pass and large deformation amount variable cross-section processing of the metal tube blank can be realized;
(2) the process flow is short and the equipment investment is small;
(3) the product has high dimensional accuracy (±0.2mm), and the surface quality of the inner wall and the outer wall is good;
(4) the process has the characteristics of forging and rolling, deformation particles are in a three-dimensional pressure stress state, and the process can be used for cold forming and hot forming of medium-small-aperture metal tubes made of various metal materials.

### Brief Description of the Drawings

Fig. 1 is a schematic view of a composite forging and rolling metal tube forming machine of the present invention;
Fig. 2 is a schematic view of a transmission of the present invention;
Fig. 3 is a schematic view of a composite forging and rolling forming device of the present invention;
Fig. 4 is a side sectional view of Fig. 3;
Fig. 5 is a schematic view of an induction heating coil of the present invention;
Fig. 6 is a schematic view of a core mold device of the present invention;
Fig. 7 is a schematic view of a feeding device of the present invention;
Fig. 8 is a schematic view of a receiving device of the present invention;
Fig. 9 is a schematic view of a medium-small-aperture thick-wall metal tube product obtained by the present invention;
Fig. 10 is a schematic cross-sectional view of Fig. 9.

Description of Reference Numerals:
1 receiving rack; 2 driving rack; 3 forming rack; 4 induction heating coil; 5 induction heating equipment control cabinet; 6 blank; 7 core mold; 8 feeding rack; 9 eccentric gear connecting rod; 10 forming rack base; 11 main driving shaft; 12 intermeshed driving bevel gear A; 13 intermeshed driving bevel gear B; 14 intermeshed driving bevel gear C; 15 intermeshed driving bevel gear D; 16 intermediate driving shaft; 17 eccentric gear shaft; 18 eccentric gear; 19 connecting shaft; 20 bearing block connecting rod; 21 sector mold block; 22 mold shaft; 23 stroke straight gear; 24 spline; 25 mold rail box; 26 feeding supporting roller; 27 hydraulic chuck; 28 servo motor; 29 decelerating pinion; 30 decelerating gearwheel; 31 chuck seat; 32 walking trolley; 33 walking trolley guide wheel; 34 positioning guide rail; 35 core mold positioning seat; 36 feeding platform; 37 supporting leg; 38 walking trolley motor; and 39 receiving supporting roller.

### Detailed Description of the Invention

The invention is further illustrated in combination with the following embodiments.

Taking steel tube 6 as a blank, the tube blank is mounted on a feeding rack 7, and the tail end of the tube blank is tightened by a hydraulic chuck 27. Meanwhile ensuring that core mold device 7 passes through the inner hole of the tube blank, the blank is fed in 25mm at a feeding speed of 1.5 m/min. The tube blank enters an induction heating coil 4 and is heated to 1000 °C and then enters a forming rack 3. Each time the tube blank is formed in the composite forging and rolling forming device, the tube blank is rotated by 60 ° around the central axis of the tube blank, and the tube blank is fed in 25mm again for forming until the front end of the tube blank enters a receiving rack 1. The receiving mechanism clamps the front end of the tube blank, while the material feeding rack releases the tail end of the tube blank. The tube blank continues to advance under the driving of the receiving mechanism until the whole tube blank is formed, and the tube blank is cooled and then cut to length.

### Embodiment 1

(1) Selecting a Q235 high-frequency longitudinal welded tube as a blank, wherein the original outer diameter of the blank is 86mm, the wall thickness is 4.5mm, and the cut length is 3m;
(2) mounting the tube blank on a feeding rack, wherein the front end of the tube blank is supported by a supporting roller, and the tail end of the tube blank is tightened by a clamping device so that the core mold device is ensured to pass through the inner hole of the tube blank and the diameter of a linear section of the mandrel is 54 mm;
(3) feeding the tube blank in by 25mm by a feeding mechanism before starting each pass at a feeding speed of 1.5 m/min, heating the blank to 1000°C by an induction heating coil, and feeding the blank into a composite forging and rolling forming device;
(4) after each forming of the tube blank in the composite forging and rolling forming device is completed, rotating the tube blank by 60 ° around the central axis of the tube blank, feeding in the tube blank by 25mm again, heating the tube blank by an induction coil, and feeding the tube blank into the composite forging and rolling forming device again for forming;
(5) repeating the process steps (3) and (4) until the front end of the tube blank enters the receiving rack, wherein the receiving mechanism clamps the front end of the tube blank while the feeding rack releases the tail end of the tube blank, and the tube blank continues to advance under the driving of the receiving mechanism until the whole tube blank is formed;
(6) cooling and shearing to length; and
the tube blank obtained by adopting the forming process having the advantages that the outer diameter is 65mm, the wall thickness is 5.5mm, the product dimensional accuracy is ± 0.2 mm, and the inner wall and the outer wall have no defects such as warped skin, pits and the like.

### Embodiment 2

(1) Selecting 08Al seamless steel tube as a blank, wherein the original outer diameter of the blank is 60mm, the wall thickness is 3.8mm, and the cut length is 5m;
(2) mounting the tube blank on a feeding rack, wherein the front end of the tube blank is supported by a supporting roller, and the tail end of the tube blank is tightened by a clamping device so that the core mold device is ensured to pass through the inner hole of the tube blank and the diameter of a linear section of the mandrel is 25mm;
(3) feeding the tube blank in by 20mm by a feeding mechanism before starting each pass at a feeding speed of 2m/min, heating the blank to 900 °C by an induction heating coil, and feeding the blank into a composite forging and rolling forming device;
(4) after each forming of the tube blank in the composite forging and rolling forming device is completed, rotating the tube blank by 75° around the central axis of the tube blank, feeding in the tube blank by 20mm again, heating the tube blank by an induction coil, and feeding the tube blank into the composite forging and rolling forming device again for forming;
(5) repeating the process steps (3) and (4) until the front end of the tube blank enters the receiving rack, wherein the receiving mechanism clamps the front end of the tube blank while the feeding rack releases the tail end of the tube blank, and the tube blank continues to advance under the driving of the receiving mechanism until the whole tube blank is formed;
(6) cooling and shearing to length; and
the tube blank obtained by adopting the forming process having the advantages that the outer diameter is 35mm, the wall thickness is 5mm, the product dimensional accuracy is ± 0.18mm, and the inner wall and the outer wall have no defects such as warped skin, pits and the like.

### Embodiment 3

(1) Selecting a purple copper tube as a blank, wherein the original outer diameter of the blank is 60mm, the wall thickness is 4mm, and the cut length is 6m;
(2) mounting the tube blank on a feeding rack, wherein the front end of the tube blank is supported by a supporting roller, and the tail end of the tube blank is tightened by a clamping device so that the core mold device is ensured to pass through the inner hole of the tube blank and the diameter of a linear section of the mandrel is 18mm;
(3) feeding the tube blank in by 10mm by a feeding mechanism before starting each pass at a feeding speed of 3m/min, and feeding the tube blank into a composite forging and rolling forming device;
(4) after each forming of the tube blank in the composite forging and rolling forming device is completed, rotating the tube blank by 45° around the central axis of the tube blank, feeding in the tube blank by 10mm again, and then feeding the tube blank into the composite forging and rolling forming device again for forming;
(5) repeating the process steps (3) and (4) until the front end of the tube blank enters the receiving rack, wherein the receiving mechanism clamps the front end of the tube blank while the feeding rack releases the tail end of the tube blank, and the tube blank continues to advance under the driving of the receiving mechanism until the whole tube blank is formed;
(6) shearing to length; and
the aluminum tube product obtained by adopting the cold forming process having the advantages that the outer diameter is 30mm, the wall thickness is 6.5mm, the inner wall and the outer wall are bright and clean, the aluminum tube product has no defects such as warped skin, pits and the like, and the dimensional accuracy of the product is ±0.2mm.

### Embodiment 4

(1) Selecting a pure aluminum tube as a blank, wherein the original outer diameter of the blank is 140mm, the wall thickness is 10mm, and the cut length is 8m;
(2) mounting the tube blank on a feeding rack, wherein the front end of the tube blank is supported by a supporting roller, and the tail end of the tube blank is tightened by a clamping device so that the core mold device is ensured to pass through the inner hole of the tube blank and the diameter of a linear section of the mandrel is 85mm;
(3) feeding the tube blank in by 8mm by a feeding mechanism before starting each pass at a feeding speed of 3m/min, and feeding the tube blank into a composite forging and rolling forming device;
(4) after each forming of the tube blank in the composite forging and rolling forming device is completed, rotating the tube blank by 25° around the central axis of the tube blank, feeding in the tube blank by 8mm again, and then feeding the tube blank into the composite forging and rolling forming device again for forming;
(5) repeating the process steps (3) and (4) until the front end of the tube blank enters the receiving rack, wherein the receiving mechanism clamps the front end of the tube blank while the feeding rack releases the tail end of the tube blank, and the tube blank continues to advance under the driving of the receiving mechanism until the whole tube blank is formed;
(6) shearing to length; and
the aluminum tube product obtained by adopting the cold forming process having the advantages that the outer diameter is 110mm, the wall thickness is 12.5mm, the inner wall and the outer wall are bright and clean, the aluminum tube product has no defects such as warped skin, pits and the like, and the dimensional accuracy of the product is ±0.2mm.

The above are the preferred embodiments of the present invention. It should be pointed out that for ordinary technologies in this technical field, several improvements and modifications can be made, without departing from the scope of the present invention as defined in the appended claims.

## Claims

1. A preparation method for medium-small-aperture thick-wall metal tube having a cross-sectional diameter in the range from 30mm to 160mm, a dimensional accuracy of ±0.2mm and a ratio of an outer diameter to a wall thickness greater than 2 to less than or equal to 20, **characterized in that** the method comprises:
(1) selecting a tube blank and cutting to length;
(2) mounting the tube blank on a feeding rack, wherein a tail end of the tube blank is tightened by a clamping device, a front end of the tube blank is supported by a supporting roller, and it is ensured that a core mold device passes through an inner hole of the tube blank;
(3) feeding the tube blank in by 5-30mm by a feeding mechanism into a composite forging and rolling forming device for forming, the composite forging and rolling forming device being composed of three swinging mold blocks, the mold blocks are arranged at equal intervals around the central axis of the tube blank at 120 °, the mold blocks synchronously swing through a crank connecting rod mechanism driven by a motor, the mold blocks rotate around a connecting shaft thereof and simultaneously do reciprocating linear movement with the connecting shaft, straight gears connected through flat keys are mounted at two ends of the connecting shaft, and moving displacement and rotating angle of the mold are controlled by the straight gears, before starting each pass, wherein the feeding speed of the tube blank is 1-3m/min ;
(4) performing a forming pass of the tube blank in the composite forging and rolling forming device and after completion, rotating the tube blank by 15-90° around a central axis of the tube blank;
(5) repeating process steps (3) and (4) until the front end of the tube blank enters a receiving rack, wherein a receiving mechanism clamps the front end of the tube blank while the feeding rack releases the tail end of the tube blank, and the tube blank continues to advance under the driving of the receiving mechanism until a whole tube blank is formed; and
(6) cooling and shearing to length.

2. The preparation method for the medium-small-aperture thick-wall metal tube according to claim 1.
**characterized in that**
in step (1), the outer diameter of the tube blank is 40-180mm and a cut length is 0.5-10m.

3. The preparation method for the medium-small-aperture thick-wall metal tube according to claim 1.
**characterized in that**
in step (3), when cold forming is carried out, the tube blank is fed and then directly fed into the composite forging and rolling forming device; when hot forming is carried out, the blank is heated to a target temperature through an induction heating device and then fed into the composite forging and rolling forming device.

4. The preparation method for the medium-small-aperture thick-wall metal tube according to claim 3.
**characterized in that**
in step (3) during the hot forming, the induction heating device is a medium-frequency induction heating coil and the target temperature range is 800-1200°C.

5. The preparation method for the medium-small-aperture thick-wall metal tube according to one of claims 1-4, **characterized in that**
the cross-sectional diameter of the metal tube ranges from 30mm to 100mm;
the ratio of the outer diameter of the metal tube to the wall thickness of the metal tube is greater than 2 to less than or equal to 12.

6. The preparation method for the medium-small-aperture thick-wall metal tube according to one of claims 1-5, **characterized in that**
the ratio of the outer diameter of the metal tube to the wall thickness of the metal tube is greater than 2 to less than or equal to 10.

7. The preparation method for the medium-small-aperture thick-wall metal tube according to one of claims 1-6, **characterized in that**
the metal tube is made of steel, copper, aluminum, magnesium, titanium or alloy.

## Patentansprüche

1. Verfahren zur Herstellung eines dickwandigen Metallrohrs mit mittlerer bis kleiner Öffnung, einem Querschnittsdurchmesser im Bereich von 30 mm bis 160 mm, einer Maßgenauigkeit von ±0,2 mm und einem Verhältnis von Außendurchmesser zu Wandstärke von größer als 2 bis kleiner oder gleich 20, **dadurch gekennzeichnet, dass** das Verfahren umfasst:
(1) Auswählen eines Rohrrohlings und Zuschneiden auf Länge;
(2) Befestigen des Rohrrohlings auf einem Zuführgestell, wobei ein hinteres Ende des Rohrrohlings durch eine Klemmvorrichtung festgeklemmt wird, ein vorderes Ende des Rohrrohlings durch eine Stützrolle abgestützt wird und sichergestellt wird, dass eine Kernformvorrichtung durch ein inneres Loch des Rohrrohlings hindurchgeht;
(3) Einführen des Rohrrohlings um 5 bis 30 mm durch einen Zuführmechanismus in eine Verbundschmiede- und Rollformvorrichtung zum Formen, wobei die Verbundschmiede- und Rollformvorrichtung aus drei schwenkbaren Formblöcken besteht, die in gleichen Abständen um die Mittelachse des Rohrrohlings in einem Winkel von 120° angeordnet sind, die Formblöcke durch einen von einem Motor angetriebenen Kurbel-Pleuel-Mechanismus synchron schwingen, die Formblöcke um eine Verbindungswelle derselben rotieren und gleichzeitig eine hin- und hergehende lineare Bewegung mit der Verbindungswelle ausführen, an beiden Enden der Verbindungswelle durch Flachkeile verbundene Stirnräder angebracht sind und die Bewegungsverschiebung und der Drehwinkel der Form durch die Stirnräder gesteuert werden, bevor jeder Durchgang gestartet wird, wobei die Zuführgeschwindigkeit des Rohrrohlings 1 bis 3 m/min beträgt;
(4) Durchführen eines Formungsdurchgangs des Rohrrohlings in der Verbundschmiede- und Rollformvorrichtung und nach Abschluss Drehen des Rohrrohlings um 15-90° um eine Mittelachse des Rohrrohlings;
(5) Wiederholen der Prozessschritte (3) und (4), bis das vordere Ende des Rohrrohlings in eine Aufnahmehalterung eintritt, wobei eine Aufnahmevorrichtung das vordere Ende des Rohrrohlings festklemmt, während die Zuführhalterung das hintere Ende des Rohrrohlings freigibt, und der Rohrrohling unter dem Antrieb der Aufnahmevorrichtung weiter vorwärts bewegt wird, bis ein vollständiger Rohrrohling geformt ist; und
(6) Kühlen und Ablängen.

2. Verfahren zur Herstellung eines dickwandigen Metallrohrs mit mittlerer bis kleiner Öffnung gemäß Anspruch 1, **dadurch gekennzeichnet, dass**
in Schritt (1) der Außendurchmesser des Rohrrohlings 40 bis 180 mm und eine Schnittlänge 0,5 bis 10 m beträgt.

3. Verfahren zur Herstellung eines dickwandigen Metallrohrs mit mittlerer bis kleiner Öffnung gemäß Anspruch 1, **dadurch gekennzeichnet, dass**
in Schritt (3) bei der Kaltumformung der Rohrrohling zugeführt und dann direkt in die Verbundschmiede- und Walzformvorrichtung eingeführt wird; bei der Warmumformung der Rohling durch eine Induktionsheizvorrichtung auf eine Zieltemperatur erhitzt und dann in die Verbundschmiede- und Walzformvorrichtung eingeführt wird.

4. Verfahren zur Herstellung eines dickwandigen Metallrohrs mit mittlerer bis kleiner Öffnung gemäß Anspruch 3, **dadurch gekennzeichnet, dass**
in Schritt (3) während der Warmumformung die Induktionsheizvorrichtung eine Mittelfrequenz-Induktionsheizspule ist und der Zieltemperaturbereich 800 bis 1200 °C beträgt.

5. Verfahren zur Herstellung eines dickwandigen Metallrohrs mit mittlerer bis kleiner Öffnung gemäß einem der Ansprüche 1 bis 4, **dadurch gekennzeichnet, dass**
der Querschnittsdurchmesser des Metallrohrs im Bereich von 30 mm bis 100 mm liegt;
das Verhältnis des Außendurchmessers des Metallrohrs zur Wandstärke des Metallrohrs größer als 2 bis kleiner oder gleich 12 ist.

6. Verfahren zur Herstellung eines dickwandigen Metallrohrs mit mittlerer bis kleiner Öffnung gemäß einem der Ansprüche 1 bis 5, **dadurch gekennzeichnet, dass**
das Verhältnis des Außendurchmessers des Metallrohrs zur Wandstärke des Metallrohrs größer als 2 bis kleiner oder gleich 10 ist.

7. Verfahren zur Herstellung eines dickwandigen Metallrohrs mit mittlerer bis kleiner Öffnung gemäß einem der Ansprüche 1 bis 6, **dadurch gekennzeichnet, dass**
das Metallrohr aus Stahl, Kupfer, Aluminium, Magnesium, Titan oder einer Legierung besteht.

## Revendications

1. Procédé de fabrication d'un tube métallique à paroi épaisse et de petit ou moyen diamètre, ayant un diamètre transversal compris entre 30 mm et 160 mm, une précision dimensionnelle de ± 0,2 mm et un rapport entre le diamètre extérieur et l'épaisseur de paroi supérieur à 2 et inférieur ou égal à 20, **caractérisé en ce que** le procédé comprend :
(1) la sélection d'une ébauche de tube et sa découpe à longueur ;
(2) la pose de l'ébauche de tube sur un support d'alimentation, dans lequel une extrémité arrière de l'ébauche de tube est serrée par un dispositif de serrage, une extrémité avant de l'ébauche de tube est soutenue par un rouleau de support, et il est assuré qu'un dispositif de moulage central passe à travers un trou intérieur de l'ébauche de tube ;
(3) l'introduction de l'ébauche de tube de 5 à 30 mm à l'aide d'un mécanisme d'alimentation dans un dispositif composite de forgeage et de laminage pour le formage, le dispositif composite de forgeage et de laminage étant composé de trois blocs de moules oscillants, les blocs de moules étant disposés à intervalles égaux autour de l'axe central de l'ébauche de tube à 120°, les blocs de moule oscillent de manière synchrone grâce à un mécanisme à manivelle et bielle entraîné par un moteur, les blocs de moule tournent autour d'un arbre de liaison et effectuent simultanément un mouvement linéaire alternatif avec l'arbre de liaison, des engrenages droits reliés par des clavettes plates sont montés aux deux extrémités de l'arbre de liaison, et le déplacement et l'angle de rotation du moule sont commandés par les engrenages droits, avant de commencer chaque passe, la vitesse d'alimentation de l'ébauche de tube étant de 1 à 3 m/min ;
(4) effectuer une passe de formage de l'ébauche de tube dans le dispositif de forgeage et de laminage composite et, une fois terminée, faire pivoter l'ébauche de tube de 15 à 90° autour d'un axe central de l'ébauche de tube ;
(5) répéter les étapes (3) et (4) jusqu'à ce que l'extrémité avant de l'ébauche de tube entre dans un plateau de réception, dans lequel un mécanisme de réception serre l'extrémité avant de l'ébauche de tube tandis que le plateau d'alimentation libère l'extrémité arrière de l'ébauche de tube, et l'ébauche de tube continue d'avancer sous l'action du mécanisme de réception jusqu'à ce qu'une ébauche de tube entière soit formée ; et
(6) refroidir et couper à longueur.

2. Procédé de préparation d'un tube métallique à paroi épaisse et de petit ou moyen diamètre selon la revendication 1,
**caractérisé en ce que**
à l'étape (1), le diamètre extérieur de l'ébauche de tube est de 40 à 180 mm et la longueur de coupe est de 0,5 à 10 m.

3. Procédé de préparation d'un tube métallique à paroi épaisse et de petit ou moyen diamètre selon la revendication 1,
**caractérisé en ce que**
à l'étape (3), lorsque le formage à froid est effectué, l'ébauche de tube est acheminée puis directement introduite dans le dispositif de forgeage et de laminage composite ; lorsque le formage à chaud est effectué, l'ébauche est portée à une température cible à l'aide d'un dispositif de chauffage par induction, puis introduite dans le dispositif de forgeage et de laminage composite.

4. Procédé de préparation d'un tube métallique à paroi épaisse et de petit ou moyen diamètre selon la revendication 3,
**caractérisé en ce que**
à l'étape (3) pendant le formage à chaud, le dispositif de chauffage par induction est une bobine de chauffage par induction à moyenne fréquence et la plage de température cible est comprise entre 800 et 1200°C.

5. Procédé de préparation d'un tube métallique à paroi épaisse et de petit ou moyen diamètre selon l'une des revendications 1 à 4,
**caractérisé en ce que**
le diamètre de la section transversale du tube métallique est compris entre 30 mm et 100 mm ;
le rapport entre le diamètre extérieur du tube métallique et l'épaisseur de la paroi du tube métallique est supérieur à 2 et inférieur ou égal à 12.

6. Procédé de préparation d'un tube métallique à paroi épaisse et de petit ou moyen diamètre selon l'une des revendications 1 à 5,
**caractérisé en ce que**
le rapport entre le diamètre extérieur du tube métallique et l'épaisseur de la paroi du tube métallique est supérieur à 2 et inférieur ou égal à 10.

7. Procédé de préparation du tube métallique à paroi épaisse et de petit ou moyen diamètre selon l'une des revendications 1 à 6,
**caractérisé en ce que**
le tube métallique est en acier, en cuivre, en aluminium, en magnésium, en titane ou en alliage.
